

Oct. 6, 1959

A. M. PARTANSKY

2,907,684

METHOD OF IMPREGNATING WOOD WITH PARAFFIN WAX AND WITH  
POLYETHYLENE GLYCOL TO IMPROVE ITS CUTTING QUALITIES

Filed April 29, 1954



Fig. 1



Fig. 2

Western incense cedar pencil slat  
having 1-6% by Wt. paraffin wax  
mostly in the spring wood and  
1-50% polyethylene glycol mostly  
in the summer wood.

INVENTOR.  
Alexander M. Partansky  
BY

Griswold & Burdick,  
ATTORNEYS

1

2,907,684

**METHOD OF IMPREGNATING WOOD WITH PARAFFIN WAX AND WITH POLYETHYLENE GLYCOL TO IMPROVE ITS CUTTING QUALITIES**

Alexander M. Partansky, Concord, Calif., assignor to The Dow Chemical Company, Midland, Mich., a corporation of Delaware

Application April 29, 1954, Serial No. 426,571

6 Claims. (Cl. 117—149)

This invention relates to a method for altering the cutting qualities of wood, to render it easier to process with saws, planers and other wood cutting tools. It relates in particular to the treatment of wood having wide natural differences in the cutting characteristics of the spring and summer wood, to equalize those properties and to make the wood substantially uniform in its behavior under the action of a knife or other cutter. It relates especially to such treatment for improving the cutting qualities of incense cedar pencilwood, and to the improved products.

The invention is not limited to use in the pencil industry, but there are problems in that industry which are of such importance that the treatment to be described herein would be fully justified even if no other use were found for it. Hence, an understanding of the pencilwood problem is desirable, and a description of the new treatment and of its effects on pencilwood will necessarily show the manner in which the same desired results may be obtained in other woods or wood products.

Wood cased pencils have been items of commerce for so long that the consuming public considers the qualities of the old standard product to be essential to a good pencil. Among the qualities as to which acceptance standards have been established through long usage are the density and whittling properties of the wood, freedom from protruding grains at the cut surface after sharpening, and the color of the freshly cut wood. The pencil manufacturer naturally desires to keep his product within the informal tolerance limits imposed by tradition, and, additionally, desires to use a wood which is easy to cut and which is sufficiently uniform to keep to a minimum the number of substandard pencils which must be rejected. Among the causes for rejection are warping, excessive softness, excessive brittleness, raised grain and failure of paint or lacquer to adhere.

The standard acceptable pencil, both from the viewpoint of ease of manufacture and from that of customer acceptance, has been made for over 100 years from eastern red cedar, *Juniperus virginiana*, grown principally in the Tennessee region of the United States. This remarkable wood is straight grained, red to brown in color, and has uniform cutting qualities because of very little difference between the hardness and density of its spring and summer wood. When cut or whittled with a knife, red cedar pencilwood gives coherent curled shavings, rather than brittle straight ones. It has a natural lubricity which appears to be lacking in the only substitute pencilwoods located to date. The need for a substitute wood has long been anticipated, however, and has become acute due to the depletion of first growth eastern red cedar and to the very inferior properties of second growth wood of this species. The latter is not straight-grained and is not uniform and cannot be used in making wood cased pencils.

Two woods have been found which have enough of the desired properties to make their use practical in pencil manufacture, but each of them has defects which must

2

be overcome if the pencils made from them are to be of high quality which has become standard. These woods are the western incense cedar, *Libocedrus decurrens*, west of the Rocky Mountains, and Kenya cedar, *Juniperus procera*, grown in and near Kenya Colony in East Equatorial Africa.

The western incense cedar is relatively free from the warping tendencies of Kenya cedar, but it presents other problems to the pencil manufacturer and pencils made from it, in its natural state, are of variable quality. Its light color is altered easily by staining to give it a color resemblance to eastern red cedar. Others of its properties are altered less easily. The difference in density between the spring wood and the summer wood of western incense cedar leads to serious problems, as it does not cut or whittle uniformly. The softer portions tend to be compressed by the cutting edge and thereafter to tear. In consequence, rough splinter ends are found on the cut surfaces. The denser layers offer temporary resistance to a cutter, requiring application of more force than when cutting the spring wood, and then, when the blade passes through the resistant summer wood it tends to lunge forward under the added force, thereby tearing the next layer of spring wood. The cuttings are not the desired coherent curls, due to the described non-uniformity. The spring wood requires stiffening and both the spring and summer woods require lubrication.

Keeping in mind the demand for pencils of uniformly high quality, an important economic problem is presented by western incense cedar. There is a great difference in the several significant properties between the sapwood and the heartwood of this tree and pencil makers have gone to the extreme of using one or the other of these and of discarding the other. Because of these differences in properties, it has become a necessary but expensive procedure to inspect every individual pencil slat made from western red cedar and to classify the slats into three or more grades. Only the top grades have been deemed useful for making acceptable quality pencils, and the waste has been appalling. Of the wood used, about 30 percent is lost as sawdust, 45 percent has been culled out as useless and only 25 percent has been useful for pencil slats, and of these, less than one-third are of the desired top grade in their natural state.

Attempts have been made in the past to overcome the above-outlined difficulties, with varying degrees of partial success. So far as is known to the world's largest pencil manufacturers and to their suppliers of pencilwood slats, no previously proposed treatment has made it possible to reproduce consistently the quality of the best grade of eastern red cedar pencils when using Kenya cedar or to make pencils of that desired quality from any but the top grade of selected western incense cedar. One of the proposed treatments for pencilwood, which has been used extensively on slats made from incense cedar, is an impregnation with paraffin wax. This stiffens the spring wood but does not appreciably lubricate the denser summer wood, and, accordingly, it has not solved the cutting problem. When used in a ratio of 13 to 20 ounces for each 13 to 13.5 pounds of western cedar (enough to make 6 gross of pencils) the spring wood cuts more easily without tearing but the wood becomes hydrophobic and difficulty is encountered in gluing and lacquering. At much lower concentrations, paraffin wax does not give sufficient improvement to the cutting characteristics of western cedar, especially of the lower grades of irregular grain to make the lower grades useful in good pencils. Paraffin wax is not useful in Kenya cedar pencil slats, as that wood does not require stiffening and paraffin exerts no significant lubricating effect to facilitate the cutting of this relatively brittle wood. The art on paraffin

impregnation of wood is too voluminous to require specific citations here.

Another treatment which has been proposed is the impregnation of wood with polyethylene glycol of molecular weight near 2000-3000 (melting point about 52° C.). Thus, Kollek et al. disclose, in U.S. Patent 1,942,146, the treatment of wood with a dilute aqueous solution of such a polymerization product of ethylene oxide, and they note that the so-impregnated wood is softer, after drying, and easier to cut than the original. The board which was treated was not identified as to species of wood. It may well be true that some woods will cut more easily if they are softened, but it is not true of woods which are suitable for making pencils. Thus, it has been found that softening agents tend to make the spring wood of western incense cedar more compressible and more prone to tear when cut, and that such an effect actually aggravates rather than eases the cutting problem. It has also been found that the lubricant needed to improve the cutting qualities of Kenya cedar should not exert much, if any, softening effect.

From the foregoing and related reasons it is desirable, and it is the principal object of the present invention to provide a method for the modification of pencilwood so that the aforementioned problems are overcome. A special object is to provide a treatment to overcome the problems peculiar to the manufacture of high quality pencils from heartwood or from sapwood of western incense cedar and to make it possible to produce pencils of substantially equal quality from grades of that wood which cannot be used either when untreated or when treated in the ways which have been proposed heretofore. Related objects include the provision of high quality pencils, equal to those made from eastern red cedar, from woods previously deemed unsuitable for such purpose. Yet another object is to provide a method for minimizing the difference between the cutting qualities of spring and summer woods of various species, to render them more broadly useful in the arts. Related objects may appear from the following description of the present invention.

According to the invention, the cutting qualities of wood are improved, without softening the wood, by a method which comprises subjecting the wood to a full cell impregnation procedure using a solution of 1 to 25 percent concentration by weight of a water-soluble polyethylene glycol, or a water-soluble ether or ester thereof, which glycol has a melting point of at least 60° C. (molecular weight at least 6000, and preferably from 8000 to 12,000), in a medium of water or other polar, water-miscible solvent, and then drying the wood slowly. The fibers of wood so-treated are permanently swollen, due to the presence therein of from 2 to 50 percent of the polyglycol. The wood cuts more easily due to the lubricating effect of the polyglycol, but is not softened by the treatment. With Kenya cedar pencilwood and with some other woods for other purposes, the polyglycol treatment with high molecular weight polyglycol is adequate to overcome the problem. (The polyglycol treatment of various woods including Kenya cedar pencilwood forms the subject of a concurrently filed application, Serial No. 426,572, now abandoned.) To make high quality pencilwood from western incense cedar, however, more is required than the polyglycol treatment if the several problems discussed above are to be overcome. Hence, in a preferred embodiment, the invention involves a multi-step treatment of western incense cedar, to be described more fully later, comprising a step of impregnation with paraffin and a step of impregnation, as above described, with aqueous polyethylene glycol, to provide 1 to 6 (preferably 3 to 5) percent by weight of paraffin and from 1 to 10 percent (preferably 2 to 6) by weight of the polyglycol, based on the weight of the air dry wood. Such a treatment stiffens the springwood, swells and lubricates all the fibers without softening them,

minimizes the differences in cutting qualities of spring and summer wood, and so nearly equalizes the properties of sapwood and heartwood, that all of the treated product is equivalent to the highest grade of pencil wood.

When the treatment is applied to western incense cedar pencilwood there is considerable latitude possible in the sequence and conditions of the treatments. The wood, usually after aging, is first cut into slats which are conventionally about  $\frac{3}{16}$  inch thick,  $7\frac{1}{4}$  inches long and of a width from "3-ply" to "8-ply," i.e., wide enough to make halves of from 3 to 8 conventional hexagonal pencils. Because of the desire for a red cedar color, the slats are stained in an aqueous dye bath using a full cell impregnation procedure. Excess liquid is drained from the slats, and they are dried slowly, over the course of 4 to 15 days or more, to prevent warping and to reach a residual moisture content near or below 10 percent. In a preferred sequence of operations, the dried slats, preferably while still warm, are dipped in or swabbed with molten paraffin or an aqueous paraffin emulsion so as to leave from 2 to 5 percent by weight of paraffin adherent to the wood. The slats are returned to an oven or kiln and held for from 3 to 6 days at a temperature slightly above the melting point of the paraffin, which becomes uniformly distributed through the wood during this heating period. Finally, the so-waxed slats are subjected to full cell impregnation with the aqueous polyglycol solution and, after draining, are slowly kiln dried as before over a period of 4 to 20 days and are ready for use in making pencils.

In an alternative sequence of operations, the polyglycol impregnation precedes that with paraffin. Since the polyglycol is absorbed in proportion to the woody fiber present, and is accordingly present in greater concentration per unit volume in the denser summer wood than in the spring wood, it is considered undesirable to effect initial dyeing or staining of the wood by putting the coloring matter in a polyglycol solution. Such a practice has the disadvantage of coloring the dense wood more heavily than the lighter wood. If the wood has been given a staining treatment before the polyglycol treatment, a deeper shade without undesirable striations may be achieved by adding dye to the polyglycol solution, and such supplemental dyeing may be done either before or after the paraffin treatment. When the paraffin is applied from aqueous emulsion, the emulsion may contain dye for a supplemental coloring treatment if desired. Examination of the treated wood reveals that the paraffin wax is found almost exclusively in the former voids or macropores of the spring wood, and is not found in the woody tissue. It is also noted that, regardless of whether paraffin is present in the wood during the treatment with polyglycol solution, the polyglycol is found only in the woody tissue which it apparently enters through micropores, and, as noted above, is distributed therein in proportion to the density of the woody tissue. Thus, maximum lubrication is available where most needed, in the denser summer wood. This selective distribution of the two agents is believed to be due to the non-polar character of the paraffin and the polar nature of the polyglycol. In view of the hydrophobic nature of paraffin wax, it was surprising that the present two-step process could be carried out successfully, and especially so that the best results are obtained when western incense cedar pencil slats are treated with paraffin before they are treated with the aqueous polyglycol. Only a small proportion of the paraffin is displaced from the wood by a subsequent impregnation with aqueous polyglycol, confirming the observation noted above that the two agents do not compete for the same position in the wood. The uniformity of cutting properties of the treated wood indicates further that each treating agent is very selective as to its site in the wood, since such results would not be obtained if each agent merely occupied a portion of

the same type of sites in a piece of wood as those occupied by the other agent.

The annexed drawing presents, as Fig. 1, a diagrammatic representation of the processes of the invention, and, as Fig. 2, a pencilwood slat having paraffin wax distributed primarily through the macropores of the spring wood and the described polyglycol compound impregnated more heavily in the dense summer wood than in the lighter spring wood, its distribution being proportional to the amount of woody fiber present.

The following examples illustrate the practice of the invention and demonstrate the importance of the several limitations as to agents for and conditions of the treatment.

#### Example 1

Western incense cedar pencil slats were impregnated with aqueous solutions of various concentrations of polyethylene glycols of various molecular weights. Impregnation was effected by immersing the slats in the treating solution in a closed vessel, reducing pressure on the vessel over the liquid until bubbles ceased to escape from the wood, then letting the slats stand overnight in the solution under atmospheric or superatmospheric pressure. The slats were so thin (about  $\frac{3}{16}$  inch) that this treatment effected full cell impregnation of the wood. The slats were drained free from adherent liquor and were oven dried. They were then conditioned at 80° F. in air at 60 percent relative humidity, to constant weight. The cutting characteristics of each batch of the treated wood were noted, and the results are tabulated below.

| Polyethylene glycol |                            |                                       |                                                                 |
|---------------------|----------------------------|---------------------------------------|-----------------------------------------------------------------|
| Molecular Weight    | Weight percent in Solution | Average percent Weight Pickup in Wood | Cutting Properties of Wood                                      |
| 1,000               | none                       | 2.3                                   | Brittle shavings; springwood compresses and tears.              |
| 1,000               | 1.0                        | 3.6                                   | No noticeable change.                                           |
| 1,000               | 2.0                        | 6.5                                   | Very little change.                                             |
| 1,000               | 3.5                        | 21.8                                  | Slight improvement, wood softened.                              |
| 1,000               | 10.0                       | 33                                    | Cuts very easily, but wood too soft.                            |
| 1,000               | 15.0                       | 4.0                                   | Too soft and sticky.                                            |
| 4,000               | 5                          | 12.8                                  | Improved, but soft.                                             |
| 4,000               | 10                         | 30.0                                  | Cuts easily, but soft and cheesy.                               |
| 4,000               | 20                         | 64.4                                  | Do.                                                             |
| 4,000               | 35                         | 95.5                                  | Excessively soft.                                               |
| 4,000               | 50                         | 6.4                                   | Do.                                                             |
| 6,000               | 5                          | 15.6                                  | Definite improvement; springwood causes knife to drag slightly. |
| 6,000               | 10                         | 19.5                                  | Much improved.                                                  |
| 6,000               | 15                         | 25.2                                  | Very good, approaches eastern cedar.                            |
| 6,000               | 20                         | 33.4                                  | Excellent, no softening.                                        |
| 6,000               | 30                         | 41.4                                  | Do.                                                             |
| 6,000               | 35                         | 66.4                                  | Do.                                                             |
| 9,200               | 2                          | 5.3                                   | Much improved, but some tearing.                                |
| 9,200               | 3.5                        | 9.3                                   | Very good.                                                      |
| 9,200               | 5                          | 12.3                                  | Closest to red cedar in properties.                             |
| 9,200               | 7                          | 21.2                                  | Very good.                                                      |
| 9,200               | 10                         | 26.4                                  | Very good, especially sapwood.                                  |
| 9,200               | 20                         | 46.3                                  | Good; possibly too easily cut.                                  |

It is noted that, using polyglycol solution as the only impregnant, no satisfactory improvement for pencilwood purposes is obtained with glycols whose molecular weight is appreciably below 6000. All lower molecular weight materials soften the wood and, as has been described, such a change is undesirable because it aggravates the problem of cutting the springwood and the undesired tearing is obtained with resultant roughness. In the tests reported above, all of the polyethylene glycols tested showed a permanent swelling effect on the wood.

In addition to the minimum molecular weight limitation derivable from the foregoing table, the useful polyglycols can be identified by their melting points, in accordance with the following table which lists the melting point and freezing point ranges of the several such glycols which are commercially available.

| Polyethylene glycol, average molecular weight |        | Melting point range, °C. | Freezing point range, °C. |
|-----------------------------------------------|--------|--------------------------|---------------------------|
| 5                                             | 1,000  | 40-43                    | 37-40                     |
|                                               | 1,540  |                          | 43-46                     |
|                                               | 2,000  | 51-54                    |                           |
|                                               | 4,000  |                          | 53-56                     |
|                                               | 6,000  | 60-63                    | 60-63                     |
|                                               | 9,000  | 64-68                    |                           |
| 10                                            | 30,000 | 65-70                    |                           |

*Note.*—The average molecular weights and the melting or freezing points are those determined and reported by commercial producers of such materials in the United States. The products from different sources differ slightly in molecular weight distribution and apparent freezing points are generally lower than melting points due to supercooling, but spot checks of the several products are in close agreement with the manufacturer's data given above.

It is apparent that, for pencil making, the treatment of western incense cedar with high molecular weight polyglycols effects a considerable improvement in the cutting qualities of the wood, but that there remains a problem in cutting the springwood without tearing it unless a very high proportion of the glycol is used. While the wood is not softened by the preferred high molecular weight polyglycols, neither is it stiffened, and some stiffening is desirable with western cedar, especially the sapwood of that species, when the wood is to be used in pencil manufacture.

#### Example 2

Previously dyes and dried incense cedar pencil slats were surface daubed with molten paraffin wax at a dosage of 8 ounces of paraffin wax for each 6 gross of pencils (about 13 pounds of wood). This represents about 4 percent of paraffin wax, based on the weight of wood. The so-treated slats were heated in a kiln at a temperature above the melting point of the wax for 5 days. The paraffin became distributed uniformly through the wood, but the treated wood did not cut easily, and shavings therefrom were brittle. The cut surfaces appeared dull, and somewhat rough, in contrast to those of eastern red cedar. Some of the paraffin treated slats were subjected to full cell impregnation with an aqueous solution of a high molecular weight polyethylene glycol, in the manner described in Example 1. After impregnation and drying, the slats had the cutting properties of eastern red cedar, showing a surface sheen on the smooth cut surfaces, and giving a coherent curled shaving. There were no noticeable differences between the ease of cutting through the springwood and the summerwood. These samples met the standards for top grade pencilwood.

#### Example 3

A mill run was made to produce enough pencil slats for 2000 gross of pencils. Western incense cedar was cut into blocks 3 x 3 x  $7\frac{1}{4}$  inches, and these were cut parallel or tangent to the annual rings to form flat slats about  $\frac{3}{16}$  inch thick. Successive slats from each block were separated into two lots of slats of as nearly equal quality as possible. After dyeing, both lots were treated with about 4 percent by weight of paraffin wax as described in Example 2. Thereafter, the slats from one lot were given a full cell impregnation using a 2 percent solution in water of polyethylene glycol of molecular weight about 9200 and melting point near 64° C. After impregnation overnight and slow drying (15 days), the glycol impregnated slats contained about 3.5 percent each of paraffin wax and the polyglycol. Both lots of slats, containing equal portions of each of several grades of wood, based on established grading practices in the trade, were shipped to a pencil factory where they were used in parallel runs on identical equipment to make wood cased pencils. The slats which had received the dual treatment with paraffin wax and with polyglycol were made into 1000 gross of pencils in 10 hours less time than was

required to make a like number of pencils from the slats treated with paraffin only. In addition, there were only 10 percent as many rejected pencils (for any cause) in the lot made from wax and polyglycol treated wood as in the lot from paraffin treated wood. The pencils from the wax and polyglycol treated wood all were of top quality, regardless of the grade classification of the wood prior to impregnation, while the only top grade pencils which were made from the wood treated only with paraffin wax were those from wood which would have been classified as of the highest quality before the wax treatment. Hence, the dual treatment of the present invention not only shortened the time required to make the pencils and reduced the number of rejects, but also gave pencils of consistent high quality.

The invention has been illustrated with respect to a particular species of wood and to the use of certain polyethylene glycols and to the application of molten paraffin wax in treating such wood to make pencil slats. It is not so limited, however. Thus, wood for art carving, or for veneers and parquetry, may be made more suitable for the purpose by impregnation with paraffin wax and polyglycols, to reduce the differences in behavior between the springwood and the summerwood. Among the woods which may be so treated for special purposes are sugar maple, white oak, yellow birch, ponderosa pine, sugar pine, redwood, cypress, Douglas fir, western hemlock and even such reformed wood products as fiberboard.

There may be used, instead of the described polyethylene glycols, aqueous, alcoholic, or acetone solutions of the ethers or esters of such glycols. Thus, the mono- and di-laurates, oleates and stearates of polyethylene glycol of molecular weight of 6000 or higher have been found to give a satisfactory degree of permanent swelling to wood when applied from solution in water or a water-miscible solvent such as ethanol or acetone, and to improve the cutting properties of the wood, and this is true whether such impregnation follows or precedes the treatment with paraffin wax. Similarly, such ethers of the polyglycols have been found useful as the mono-allyl ether, the mono-sec. butylphenyl ether and the monoethyl ether.

When any of the polyglycol compounds suggested above is being used, and it is desired to increase the hardness of the wood, there may be added to the solution of the polyglycol a wood hardener which is soluble in the same medium. Examples of such hardeners are the aldose and ketose sugars, such as glucose, fructose and lactose, and any of several water-soluble resins, especially those which tend to harden during exposure to enough heat to dry the impregnated wood. Among the resins and polymers which may be used are water-soluble phenol-formaldehyde resins, water-soluble urea- or melamine-aldehyde resins, toluene sulfonamide-aldehyde resins, and water-soluble polymers, such as polyacrylamide, polyacrylic acid, polyvinylalcohol and polyvinylsulfonic acid.

The following examples illustrate the effect of typical hardening agents when used together with a polyethylene glycol. In these examples, no paraffin wax treatment was used, as it is desired only to demonstrate the effect of the hardener.

#### Example 4

Pencil slats of incense cedar sapwood and heartwood and of Kenya cedar were impregnated in similar manner with mixed aqueous solutions of varying composition containing polyethylene glycol (mol wt. 6000) and a phenolformaldehyde resin as hardener. The resin was made from a mixture consisting of 349 grams (3.71 mols) phenol, 550 cc. (7.42 mols) 37 percent aqueous formaldehyde solution, 17.5 grams sodium carbonate, 17.5 grams alpha-protein and 3 grams added water, which was cooked under reflux to a viscosity of 50 centipoises. The following table shows the composition of the treating solutions in percentage by weight and the increase in dry weight of the treated samples.

| 5  | Solution:          |               | Percent Gain in Weight |           |       |
|----|--------------------|---------------|------------------------|-----------|-------|
|    | Percent Polyglycol | Percent Resin | Sapwood                | Heartwood | Kenya |
| 10 | 5.0                | 1.8           | 20.0                   | 17.0      | 6.0   |
|    | 7.0                | 2.5           | 17.0                   | 18.0      | 5.0   |
| 15 | 10.0               | 3.5           | 27.0                   | 33.0      | 7.0   |
|    | 15.0               | 7.5           | 66.0                   | 47.0      | 14.0  |

All of the treated samples showed excellent cutting properties, superior to the untreated wood, except the incense cedar sample containing 66.0 percent added solids, which was too hard and "gritty" for good cutting.

#### Example 5

To show the hardening effect of dextrose, test blocks of incense cedar sapwood and heartwood were impregnated with 15 percent aqueous solutions of polyethylene glycol (mol wt. 9000) to which varying amounts of commercial dextrose were added. The samples were weighed to determine gain in weight, and their cutting properties tested, with results as given in the following table.

| 30 | No. | Percent Dextrose in Soln. | Percent Gain in Weight |           | Cutting Properties |
|----|-----|---------------------------|------------------------|-----------|--------------------|
|    |     |                           | Sapwood                | Heartwood |                    |
| 35 | 1   | 1.0                       | 37.0                   | 21.0      | Slightly soft.     |
|    | 2   | 2.0                       | 40.0                   | 34.0      | Excellent.         |
| 40 | 3   | 3.5                       | 43.0                   | 25.0      | Very good.         |
|    | 4   | 5.0                       | 47.0                   | 33.0      | Slightly too hard. |

Incense cedar, when impregnated with a 15 percent solution of polyethylene glycol (mol wt. 9000) is somewhat too soft for best cutting properties. When the treating solution is modified by addition of small amounts of dextrose, as above, the hardness of incense cedar impregnated with the modified solution is increased. Of the above samples, No. 1 is slightly too soft, Nos. 2 and 3 have a degree of hardness giving desirable cutting properties, and No. 4 is slightly too hard.

The paraffin wax which is used in the treatment of wood according to the present invention is any such wax having a melting point of 120° F. (49° C.) or higher. It may be applied, as described, from the molten condition, or it may be used in the form of an aqueous emulsion, either type of application being followed by heat treating the wood to cause the wax to melt and to become uniformly distributed through the wood in which it is found thereafter to be principally in the springwood. The paraffin wax treatment is preferably employed before the wood has been impregnated with the high molecular weight polyglycol, but it has been found that the cutting properties of western incense cedar pencilwood are improved to substantially the same extent when the paraffin wax treatment follows the treatment with the polyglycol.

The specific conditions employed in the successive treating steps of the invention do not appear to be critical so long as the paraffin wax is so applied as to become substantially uniformly distributed through the wood and the polyethylene glycol is used in any of the well known full cell impregnation procedures. When applying the invention to western incense cedar pencil slats it is important that the wood be dried very slowly after any impregnation with an aqueous solution, to prevent warping and to prevent the escaping water from carrying its solute to the surface of the wood. Similar considerations recommend a slow drying procedure when the invention is applied to woods other than incense cedar which tend to warp or to display raised grain after treatment with aqueous media.

The amount of paraffin wax and of polyglycol needed to give the maximum reduction in the differences between cutting properties of spring and summer wood

varies somewhat with the species being treated. The amount of paraffin wax which can be used advantageously seldom exceeds 6 percent of the weight of wood, and is often as little as 1 to 2 percent, though there are uses for various woods in which larger amounts of paraffin are not harmful. The amount of polyglycol varies more widely, being most frequently in the range from 2 to 10 percent, with amounts up to 50 percent being acceptable in the case of some light, brittle woods.

I claim:

1. The method for diminishing differences between the cutting characteristics of spring and summer wood without materially softening the wood, which comprises the steps of (A) distributing through the wood from 1 to 6 percent of its weight of paraffin wax having a melting point of at least 49° C.; and (B) subjecting the wood to full cell impregnation with a water-miscible solution of from 1 to 25 percent by weight of a compound from the group consisting of polyethylene glycol, having a molecular weight of at least 6000 and a melting point of at least 60° C., and the water-soluble ethers and esters thereof, and drying the so-impregnated wood slowly.

2. The method claimed in claim 1, wherein the wood subjected to treatment is western incense cedar.

3. The method claimed in claim 1, wherein step (A) precedes step (B).

4. The method claimed in claim 1, wherein step (B) is carried out using a water solution of from 1 to 5 percent concentration by weight of polyethylene glycol having a molecular weight of from 6000 to 12,000 and a melting point of at least 60° C.

5. The method which comprises distributing substantially uniformly through western incense cedar pencil slats

from 1 to 6 percent of their weight of paraffin wax having a melting point of at least 49° C. and thereafter subjecting the slats to full cell impregnation with a water solution of from 1 to 5 percent concentration by weight of polyethylene glycol having a molecular weight of from 6000 to 12,000 and a melting point of at least 60° C., and drying the so-impregnated slats slowly so as to avoid warping, thereby to minimize differences between the cutting characteristics of spring and summer wood.

10 6. The method of diminishing differences between the cutting characteristics of spring and summer wood without materially softening the wood, which comprises the steps of impregnating the wood with paraffin wax so that the wax enters the voids and pores thereof, impregnating the wood with an aqueous solution of polyethylene glycol having a molecular weight of from about 6000 to 12,000 and then slowly drying the so impregnated wood.

References Cited in the file of this patent

UNITED STATES PATENTS

|           |                |               |
|-----------|----------------|---------------|
| 997,275   | Crocker        | July 11, 1911 |
| 1,699,635 | Smith          | Jan. 22, 1929 |
| 1,942,146 | Kolleck et al. | Jan. 2, 1934  |
| 2,386,828 | Wilcox         | Oct. 16, 1945 |
| 2,469,049 | Miller         | May 3, 1949   |

FOREIGN PATENTS

|         |        |              |
|---------|--------|--------------|
| 831,524 | France | June 7, 1938 |
|---------|--------|--------------|

OTHER REFERENCES

"Wood Preservation," B. Van Groenou, Holland, 1951.  
(Copy in Div. 25.)